

# UNITED STATES PATENT OFFICE.

CHARLES SCHWARTZ, OF VILLEURBANNE, FRANCE, ASSIGNOR TO SOCIETE GILLET & FILS, OF LYON, RHÔNE, FRANCE, A CORPORATION OF FRANCE.

## PROCESS FOR THE TREATMENT OF VEGETABLE FIBERS.

1,398,804.

Specification of Letters Patent. Patented Nov. 29, 1921.

No Drawing.

Application filed December 9, 1919. Serial No. 343,576.

To all whom it may concern:

Be it known that I, CHARLES SCHWARTZ, a citizen of the Republic of France, and a resident of Villeurbanne, Department of Rhône, France, have invented a new and useful Process for the Treatment of Vegetable Fibers, of which the following is a specification.

There is an already known process for dressing or glossing textile fabrics, which consists in impregnating them with a solution of cellulose in zinc chlorid and precipitating the cellulose upon the vegetable fiber by subsequent washing of the zinc chlorid (German Patent No. 84,513).

It has also been proposed to impart to cotton a luster similar to that of silk by treatment with alkaline solution of nitrocellulose (German Patent No. 98,602).

20 The present process for treating vegetable fibers is intended—to impart to them the character of wool, both physically as to the feel, appearance and caloric qualities and chemically as regards their affinity and absorption capacity for dyestuffs.

This process is applicable to vegetable fibers of all kinds, in the raw state or bleached, and whether mercerized or not, at any stage whatever in the operations to 30 which they are subjected in the textile industry, either in the mass, or in the state of waste, lap, fleece, card-ends, yarns or fabrics.

This process consists in impregnating these vegetable fibers by means of a solution 35 of cellulose, of any origin, in concentrated nitric-acid preferably of a concentration equal to or higher than 65 per cent., and in precipitating upon the fibers a slightly nitrated cellulose by washing these treated 40 fibers by means of water. The product which is deposited upon the fiber contains about 5 to 6 per cent. of nitrogen.

It has been found that this precipitation of the nitrocellulose is more rapid and complete if, instead of treating the fibers soaked in the solution with water, they are treated with dilute solutions of acids or bases or with saline solutions. The use of sulfuric acid, for example, or ammonia, sodium bisulfate, ammonium sulfate, sodium sulfate, or sodium phosphate in 10 per cent. aqueous solutions, will give good results.

The textile material impregnated with a solution of cellulose in nitric acid, is to be

treated with one of the baths indicated above, 55 and then washed with water. The precipitation of nitrocellulose upon the vegetable fibers takes place instantaneously and, owing to this rapid action, the fibers absorb the substance better. Moreover the final washing is quicker and the recovery of the nitric acid is facilitated.

The temperature of the cellulose solutions may be from 0° to approximately 25° centigrade, and the duration of contact may 65 vary within limits up to half an hour with corresponding concentrations of nitric acid, without any disadvantage as regards the result of the reaction.

The textile material remains sound and 70 strong during the operation; this solution in excess may be expelled by pressure and the textile washed.

After pressing and washing the textile fiber, the nitrocellulose remains firmly adherent to the steeped fiber and is definitively combined with the latter, forming a union which resists any mechanical or chemical operation which the treated fiber may have 75 further to undergo.

The nitrocellulose absorbed by the fiber and precipitated upon and within the same, behaves thereafter quite differently from the case of a dressing or gloss upon the fiber.

The inflammability of the textile material 85 when treated and dried is scarcely increased at all, so that there is no objection to its direct utilization. Denitration in accordance with one of the known processes is not therefore necessary, but, if applied to certain 90 kinds of fabrics treated by this process, it increases the wool-resembling character of the material.

The weight of deposit is greater or less 95 according to the content of cellulose-matter in the solution. It is to be noted that the use of celluloses, mercerized by alkalis or by acids or hydrolyzed, increases the solvent and absorbent power of the nitric acid.

The strength of resistance of the treated 100 fiber is considerably increased by the process forming the subject of the invention. The absorption of nitrocellulose produces moreover a large increase of weight and in fabrics a much denser gloss. The dye-absorbing 105 power is much higher, even as regards basic colors, which dye the treated vegetable fiber easily and without the use of a mordant.

The entire character of the textile material is profoundly modified by this process; it is denser, has more body and is moreover more supple, becoming generally of the nature of wool.

This process of treatment is equally advantageous for lap or fleece as for drawn stuffs and fabrics of all kinds, without distinction of quality, whether plain, ornate 10 or worked.

Print-effects may also be obtained upon plain or drawn stuffs, either by direct impression, the fabric being impregnated with the cellulose solution at the desired parts 15 and the nitrocellulose then precipitated at these parts by washing, or by the use of suitable resists or reserve pastes, such as kaolin, at the parts where the print-effects are to be avoided, and by treatment with the 20 cellulose solution and precipitation by washing of the other parts.

The solution employed for the treatment of textile materials may for example be prepared in the following manner:

25 I. Introduce rapidly and with constant stirring, 30 grams of wood-pulp or cotton-waste, the whole being thoroughly disintegrated and bleached, into 1000 grams of 81 per cent. nitric acid, at a temperature of 15 30 to 20° centigrade; after complete solution to a syrupy mass, add 112 grams of water.

II. Proceed as above, dissolving 50 grams of mercerized cellulose in 1000 grams of 83 per cent. nitric acid, and then add 250 grams 35 of water.

III. Prepare a solution as above, by dissolving 100 grams of hydrocellulose in 1000 grams of 81 per cent. nitric acid, and adding 112 grams of water.

40 IV. Introduce 70 grams of mercerized cellulose into 750 grams of 75 per cent. nitric acid; leave for two hours and then remove about 460 grams of acid by decantation and pressure. Add the residue to 500 grams of 45 92 per cent. nitric acid, or vice versa, solution being instantaneous, and then add 145 grams of water.

The viscous solutions prepared as above are allowed to cool to 15 to 20° centigrade, 50 and are kept in a cool place.

The treatment of the vegetable fibers is effected by introducing the textile material into the liquid of syrupy consistency, in which it is left for a certain time without

tension; the liquid is then pressed or dried out and the material washed.

Solutions prepared in accordance with paragraphs I, III and IV are intended for fabrics of inferior quality (American cotton); the solution prepared according to 60 paragraph II is intended for use with fabrics of better quality, such as batiste (Egyptian cotton).

The time of impregnation of the textile material with the solution is in general 3 65 to 5 minutes, according to the nature and permeability of the material; it may be extended to half an hour without harm to the final result, provided the temperature of the cellulose solution employed does not exceed 70 20° centigrade.

The reaction takes place as easily at 0° as at 25° C., but since the solutions become more and more viscous with the fall of temperature, it is advantageous in practice to 75 work at a temperature of 12° to 30° C.

Having now particularly described and ascertained the nature of my said invention, and in what manner the same is to be performed, I declare that what I claim, is:—

1. A process for the treatment of vegetable fibers with a view to impart to them the character of wool, both physically, as to the feel, appearance and caloric quality, and chemically, as regards their affinity and 80 absorbent capacity for dyestuffs, said process consisting in impregnating the fiber with a solution of cellulose in concentrated nitric acid, and precipitating upon the fiber a slightly nitrated cellulose by washing with 90 water.

2. A process for the treatment of vegetable fibers with a view to impart to them the character of wool, both physically, as to the feel, appearance and caloric quality, and 95 chemically, as regards their affinity and absorbent capacity for dyestuffs, said process consisting in impregnating the fiber with a solution of cellulose in concentrated nitric acid, at a concentration of at least 65%, and 100 in precipitating upon the fiber a slightly nitrated cellulose by washing with water.

In testimony whereof I have signed my name to this specification.

CHARLES SCHWARTZ.

Witnesses:

PHILIPPA DEOGRANGAS,  
ADOLPHE BOHN.